

May 16, 1944.

W. B. WESCOTT

2,348,943

PLANOGRAPHIC PRINTING PLATE

Filed April 28, 1943



Fig. 1



Fig. 2



Inventor  
William B. Wescott  
by Polk, Cushman, Hardway  
Attnys.

## UNITED STATES PATENT OFFICE

2,348,943

## PLANOGRAPHIC PRINTING PLATE

William B. Wescott, Dover, Mass., assignor to  
Addressograph-Multigraph Corporation, Wil-  
mington, Del., a corporation of Delaware

Application April 28, 1943, Serial No. 484,833

9 Claims. (Cl. 101—149.2)

This invention relates to planographic printing and more particularly to a parchmentized cellulose planographic printing plate, and this application is a continuation-in-part of my copending application Serial No. 471,673, filed January 8, 1943. My prior patents, Nos. 2,224,370, 2,134,165 and 2,205,998 may be referred to as showing the state of this art.

Parchmentized cellulose planographic printing plates offer numerous advantages over the older planographic printing plates of metal by reason of their flexibility and ease of handling in a typewriter, rendering them particularly adapted to office use in connection with cylinder offset reproducing machines. However, the use of parchmentized cellulose printing plates, though extensive, has been limited in certain respects. Their use could have been greatly enlarged were it not for two conditions that have not heretofore been overcome, namely, (1) the very short useful life of unbacked parchmentized cellulose printing plates, and (2) the difficulties, expense, and complications encountered in making and handling the prior parchmentized cellulose printing plates having backing layers.

The very short useful life of unbacked parchmentized cellulose printing plates arises from the fact that they must absorb water as they are used in planographic printing, and that as they absorb water they expand rapidly, principally in width. After a very few impressions such unbacked parchmentized cellulose plates show considerable distortion of the image and loss of sharpness of the image, rendering them unfit for further use.

Backed plates consisting of parchmentized cellulose, a backing layer, and an intermediate bonding layer of water-impermeable adhesive, prevent lateral expansion of the printing surface but are subject to a number of difficulties. Provision of a non-extensible backing for the parchmentized cellulose printing layer prevents the undesired lateral expansion, but this expedient introduces a number of difficulties.

Operation of the parchmentized cellulose as a planographic printing element depends upon its printing surface being water-receptive at all places excepting where grease-receptive image-forming material has been applied to make its image area non-receptive to water. To retain the backing firmly adherent to the parchmentized cellulose when the latter is moist requires an adhesive which is relatively water-impermeable. All such water-impermeable adhesives are necessarily preferentially grease-receptive rather

than water-receptive, and on the surface of the plate would behave as a grease-receptive contaminant. Parchmentized cellulose is to some extent permeable to the adhesive. A high degree of pressure is necessary in order to obtain the requisite degree of adhesion between the parchmentized cellulose and the backing layer. This pressure tends to force the adhesive both through the backing layer and through the parchmentized cellulose. This effect is heightened by the necessary presence of plasticizers in the adhesive, the suitable plasticizers also acting as contaminants of the printing surface. Because of tiny pinholes which characterize thin parchmentized cellulose and provide paths through which the adhesive can flow toward the printing surface, it is found impractical to use parchmentized cellulose sheets of less than 50 pounds ream weight (24 x 36—500 basis) for the printing surface in backed parchmentized cellulose plates.

In order to minimize the migration of the contaminating adhesive to the face of the printing surface it is customary to use a greater thickness or weight of parchmentized cellulose than is needed as a printing element. Fifty to sixty pounds ream weight has been found to be the minimum satisfactory weight, whereas if it were not for the contamination by the adhesive of sheets of that weight, twenty-five to thirty pounds would be satisfactory.

Contamination of the printing surface may also occur as a result of pressure contact of the printing face of one sheet with the backing of another, and the complete avoidance of such contamination requires special steps in manufacture and handling as more fully described in my copending application Serial No. 312,390, filed January 4, 1940.

Objects of the present invention are to avoid the above difficulties and disadvantages, to provide a parchmentized cellulose printing element that is cheaper than the previous backed elements, and with which it is easy to avoid contamination in manufacture and handling. These and further advantages are attained by the present invention which will now be described.

The invention involves the discovery that by taking two sheets of cellulose water leaf, each 50 in the process of being acted on by the acid in parchmentizing, at least one being adapted to serve as a planographic printing surface upon washing and drying, and then in a manner known in the making of laminated parchment, laminating and cohering these together while

under the influence of the acid and washing the acid therefrom, and drying, there can be made a sheet which is admirably suited to be cut into planographic printing plates. There is no tendency, either originally or later, for the printing surface of the plate to be contaminated by adhesive, since the junction between the two sheets is formed of the same material as the printing surface and is free of extraneous bonding agents. The plates are much cheaper in cost than previous backed printing plates. The involved step of applying an adhesively secured backing is avoided. The material requires less handling in its manufacture. No special requirements exist as to packing the plates. Yet compared to plates of equal weight and equal surface-parchmentization but composed of a single thickness of parchmentized cellulose, the new plates take four to ten times as long to expand a given amount in width in use on an offset planographic press and hence will make four to ten times as many good impressions in printing.

In the drawing,

Fig. 1 is a perspective view of a printing plate made in accordance with the present invention;

Fig. 2 is an enlarged fragmentary edge view of the printing plate of Fig. 1; and

Fig. 3 is a schematic view indicating the principal steps in manufacturing the material of the printing plates of the present invention.

Referring to Fig. 2, the material of the printing plate consists entirely of cellulose, consisting in part of the fibrous form of cellulose and in part of the amyloid non-fibrous form of cellulose resulting from the parchmentizing process. Among the known characteristics of parchmentized cellulose suitable for use as a planographic printing plate are: that it readily receives and retains the ink-receptive image-forming material (of which numerous examples are known to the art and further examples are set forth in my copending application Serial No. 312,391, filed January 4, 1940); that it is readily wet by and absorptive of water; and that it is free from any added component or contaminant which either causes the printing ink to displace water previously applied or causes water later applied to displace the ink-receptive image-forming material which has been initially applied to the dry sheet. The sheet is relatively strong and is highly resistant to disintegration by water.

As shown in Fig. 2 both the outer printing face 11 and the corresponding rear face 12 are each constituted of non-fibrous amyloid cellulose overlaying the cellulose fibers. Inwardly of the printing face 11 and inwardly of the rear face 12, the non-fibrous amyloid cellulose, represented by the stippling in Fig. 2, becomes less dense, there forming a net-work which is integral with the amyloid cellulose on the surface and is bonded to the cellulose fibers with which it is intermingled. Finally, in a stratum extending through the middle of the thickness of the sheet the net-works of amyloid cellulose of the upper and lower halves are integrally joined by a dense stratum 13 of the same amyloid cellulose, free from fiber. The whole plate thus consists of unified cellulose, contains fibers in its two halves and has extending throughout the plate a continuum of non-fibrous amyloid cellulose which overlays the fibers near each face of the plate and also forms a fiber-free and dense stratum at its junction between the two constituent sheets.

An example of the preferred procedure in pro-

ducing the material for this planographic printing plate is as follows:

Two webs 20 and 21 of unsized paper or waterleaf made from bleached sulphite stock, free from any of the undesirable added components or contaminants as explained above, are simultaneously subjected to a conventional parchmentizing treatment in a sulphuric acid bath 23. Upon emerging from the bath and while their surfaces are still in the gelatinous state induced by the acid and still wet thereby, the two webs 20 and 21 are led into contact face to face and passed between a pair of press rolls 25 and 26 which subject the webs to a pressure sufficient to effect a firm fusion of the contacting cohering gelatinous surfaces of the webs. The acid and water are removed by passing the composite web through any suitable washing apparatus 27 and drying apparatus 28.

The unified sheet thus produced is then cut up into printing plates which are provided with any desired structure at their ends for attaching them to the printing machine. As shown by way of example in Fig. 1, front and rear edges 38 of each sheet may for example be cut in a sinusoidal shape and provided with elongate perforations 33 to permit convenient attachment to the printing machine.

Referring again to Fig. 2, the opposite faces 30 of the plate consist of a continuum of the non-fibrous amyloid form of substantially pure cellulose. The middle stratum of the plate likewise consists of the same continuum of non-fibrous amyloid form of cellulose, and since it was formed 35 by the union of gelatinous faces of the two original webs, is substantially free of any fibrous form of cellulose. Nevertheless this middle stratum is thoroughly bonded to all of the remainder of the plate by the extension outwardly 40 from this middle strata of less dense but unitary amyloid cellulose bonded to the individual fibers remaining from the two original webs.

As shown in Fig. 2, the thickness of the middle stratum 13 of fiber-free cellulose is greater than 45 the sum of the two thicknesses of the fiber-free cellulose which overlay the fibers near the two faces 11 and 12. As the composite web 20, 21 is washed, the parchmentizing action is checked more quickly at the two outer faces of the web 50 than in the middle zone where the webs are joined. This is advantageous in permitting a relatively thick middle stratum of amyloid cellulose to be formed without causing either the printing face or the back face of the plate to be unduly or unnecessarily parchmentized.

The plate is water-absorptive, as it must be to function as a parchmentized cellulose planographic printing element. The plate tends to expand as it absorbs water during the printing, but surprisingly the increase in dimension due to absorption of water takes place, in its initial stages, at a much slower rate (one-fourth to one-tenth) than in the case of a plate of equal weight and surface-parchmentization consisting of a single layer of parchmentized cellulose. Accordingly, within the limitation of the desired good quality of the impressions, four to ten times as many good impressions can be made.

The plate constitutes a valuable improvement over previous backed plates of parchmentized cellulose. There is no tendency of the absorbed water to weaken the bond between the front and back of the sheet. All tendency toward contamination of the printing surface by adhesive bond-

ing of the front to the back of the plate is avoided. The junction between the two halves of the plate is formed of the same amyloid cellulose that is employed as the printing face. No plasticizer is needed in effecting this junction, since use is made of the cohesive bonding tendency of cellulose when in the active gelatinous state. All difficulties with contamination of the printing surface by plasticizers are avoided.

It is no longer necessary to increase the thickness of parchmentized cellulose for the printing element for the purpose of guarding against migration of adhesive and its plasticizer to the printing surface. Thinner sheets may accordingly be used without any resulting contamination. For instance, the two webs 20 and 21 which are bonded together to form the material of the plate each may advantageously have a ream weight (24 x 36—500 basis) of as low as 25 pounds.

The back of the plate cannot exert any contaminating effect of the face of another plate with which it may contact for as indicated above, no added adhesive is applied and hence none is present to permeate the back of the sheet.

An advantage of the present invention is that the aggregate hardness of the printing plate is substantially greater than the aggregate hardness of a plate of equal total thickness consisting of a front layer of parchmentized cellulose, an intermediate bonding layer, and a backing layer of kraft paper, the hardness of the parchmentized cellulose being substantially greater than that of kraft backing paper. This increased aggregate hardness of the plate results in a crisper image, particularly in typewriting upon the plate.

It is recommended that the two component faces of the plate be approximately balanced as to density, that is, contribute substantially equally to the total density of the plate, in order that the plate may have as little tendency to curl as possible.

The expression "density" is herein used in reference to the compactness of the parchmentized cellulose. Density of parchmentized cellulose varies with, and may be satisfactorily expressed in terms of, translucency or opacity, bearing in mind the fact that the opacity of a sheet of given density varies with the thickness so that numerical values of opacity reflect comparative densities only for sheets of the same thickness.

Within the limits of surface smoothness which are recommended, and provided the plate is of substantially uniform opacity throughout its area, the opacity of the parchmentized cellulose printing plate of this invention is a satisfactory criterion of density of the plate as a whole. A parchmentized cellulose printing plate of the present invention having a surface smoothness of from four to eight as determined by the Bekk smoothness tester and of 60 pound ream weight and about 0.004 inch in thickness should in order to have the proper density, have an opacity, as determined by the Bausch & Lomb opacimeter, of not over 0.60; the opacity of this same plate should also preferably be not less than 0.45 because lower opacities than 0.45, at this thickness, indicate such a high degree of parchmentization as results in too great brittleness for convenient handling. Plates of other thicknesses should have the density of the plate just described, the values of opacity corresponding to such density and the plate thickness.

The outer printing face 11 should, for typewriting and crayon work, have a smoothness of two or upwards, as determined by the Bekk smoothness tester; while for penmanship, whether writing or line drawing, the smoothness should be four or more. Although satisfactory results can be obtained at values corresponding to glossy surfaces, a smoothness in the optimum range of from four to eight is preferred.

10 In order to absorb the dampening solution in planographic printing the parchmentized cellulose of the outer printing face 11 necessarily has a positive absorption for water. But an advantageous improvement in life of the image 15 under printing conditions occurs if, as is preferred, the outer printing face has a rate of lateral water diffusion of not more than 25 millimeters in four hours, while having the characteristics of density and smoothness as 20 above described. The lateral water diffusion rate herein referred to means the result of a test (as later herein described) of the sheet in its normal condition of inherent density, and not while in a temporarily altered condition of 25 density which would result, for example, from calendaring the sheet after formation, it being well known that calendaring may give the sheet increased density, decreased porosity, and a changed diffusion rate, all of which characteristics 30 may be restored to normal by soaking and drying the sheet.

For the present purpose the lateral diffusion rate of water in unified cellulosic material is defined as the height (expressed in millimeters) to 35 which distilled water rises in a sheet of said material over a period of 4 hours when the edges thereof are sealed against absorption of water in any convenient manner and when the sheet is suspended over a quiescent bath of said water at 40 room temperature under the following further conditions: (1) the lower end of the sheet is maintained below the level of the bath, this being conveniently accomplished by folding a bit of sheeted block tin over the bottom edge; (2) 45 the machine direction of the sheet is to be parallel to the surface of the bath; (3) the portion of the specimen above the bath is surrounded by moisture-saturated air; (4) a marker having been inscribed at the edge of the sheet, the sheet 50 is submerged for 1 minute to exactly this mark and then raised by an amount slightly greater than the expansibility of the sheet in a direction normal to the machine direction thereof; (5) the sheet is suspended thus for 4 hours, at the end 55 of which time the rise from the marker is measured off in millimeters.

A preferred way of causing the parchmentized cellulose to have the desired low rate of lateral water diffusion, without loss of the desirable 60 characteristics as to density and smoothness, consists in an accelerated oxidation of the surface of the material of the plate.

The increment in oxidation-products content due to such accelerated oxidation may be employed as a useful measure of the effectiveness of the accelerated oxidation. (By oxidation-products content is here meant the sum of the copper number and percentage cold alkali solubility.) It is recommended that the accelerated 65 oxidation be carried on to such extent that the increment in oxidation-products content due to such accelerated oxidation will be at least 10% over that of the material of the plate as freshly made. Improvement in press performance may 70 be expected to result from still greater increase 75

in oxidation products content due to accelerated oxidation, but the accelerated oxidation should not be carried so far as to cause marked discoloration or brittleness.

Accelerated oxidation of the surface of the material of the plate may be brought about in a number of ways in which the surface of the plate is accessible to air, oxygen or ozone. For example, exposure to sunlight is effective but is not recommended as a commercial procedure. Exposure to artificially produced ultra violet light is effective. Ultra violet irradiation at 10 inches from a quartz mercury vapor arc lamp for from 2 to 15 minutes, depending upon the reactivity of the stock being treated, will suffice. Other known ways of oxidizing cellulose, including the application of non-gaseous oxidizing agents thereto, have been tried and found to yield more or less satisfactory results.

A suitable method of predisposing the surface to accelerated oxidation by contacting the surface with anhydrous chlorine gas is disclosed in my said copending application Serial No. 312,390, which may be referred to for details of such step. Following such predisposition to accelerated oxidation the desired increase in oxidation-products content will take place upon mere exposure of the surface to air for a time of the order of 1 to 3 weeks.

I have discovered that resinous extractives contained as inevitable impurities in commercially available wood pulp tend to be the cause of ink-retentive spots which develop autogeneously on the surface of the plate. To minimize such effect, it is desirable to take two precautions. Firstly, the material from which the outer printing face is made is preferably initially selected from material which does not contain more than 0.5% of resinous extractives. Although some appreciable quantity of resinous extractives will be found in all commercial grades of paper-making wood pulp available for manufacture of the plates, this requirement of an upper limit of 0.5% of resinous extractives can be met by the better grades of the paper-making wood pulp which is commercially available. Although a certain amount of resinous extractives is inevitable, and such resinous extractives exist as tiny particles within the material of the plate, the parchmentizing process has the effect of preventing any substantial number of these particles from initially being located at the printing surface of the plate. Apparently during the parchmentization the cellulose gel at and near the surface flows over and forms a continuum covering substantially all of the particles of resinous extractives which might otherwise be exposed at the surface of the plate.

But the cellulose of the printing plate is permeable to resinous material in the normal mobile condition of the resinous material. Traces of such mobile resinous material initially contained in the body of the plate tend to migrate through the non-fibrous surface continuum and finally appear on the printing surface of the plate. Even such traces of resinous material, when exposed on the surface of the plate, become ink-receptive and ink-retentive. Therefore, as a second precaution, it is preferable to immobilize the traces of resinous extractives contained in the printing face of the material of the plate and thereby prevent them from migrating to the printing surface. The resinous extractives may be thus immobilized by sufficiently aging either the wood pulp from which the waterleaf is made,

or the waterleaf itself, or both, either naturally or accelerated by heat or other means before the parchmentizing operation. The sufficiency of such aging and the practical freedom of the

plate from tendency to form ink-retentive spots due to resinous material at its printing surface may be ascertained by an accelerated test of the printing plate comprising incubating the plate for 4 days at 150° F., irradiating the printing face by ultra violet light from a quartz mercury vapor arc lamp (Hanovia type) for 15 minutes at a mean distance of 10 inches, thoroughly saturating the printing surface with the etching solution described in my United States Patent No. 2,003,268, dated May 28, 1935, comprising ammonium dihydrogen phosphate, nickel or cobalt nitrate, glycerin and water, removing any superficial etch with blotting paper or the like, and then immediately rolling up a portion of the so-dampened surface with a usual stiff offset lithographic printing ink. As a result of this test, the macroscopically discernible pinpoint ink-retentive spots should not on the average be more than 0.5 millimeter in diameter and not of greater occurrence than one such spot for each square inch of plate surface.

Of course it is possible, and may sometimes be desirable to have both faces of the plate consist of identical material. But, when only one face has the preferred characteristics as to surface smoothness, low lateral water diffusion rate, low content of resinous extractives and substantial immobility of the resinous extractives, and is thus to be the only face intended for printing, then it is desirable to differentiate the two faces by giving one or the other a trace of coloring so that the face intended as the printing face will be instantly apparent.

I claim:

1. A parchmentized cellulose planographic printing plate, the printing surface thereof having planographic printing characteristics, and the plate being formed of two superposed sheets of parchmentized cellulose, a continuum of non-fibrous amyloid cellulose extending throughout both sheets, said continuum overlaying the fibers near each face of the plate and also constituting a fiber-free and dense stratum at the junction between the two sheets, said junction stratum integrally uniting the two constituent sheets and being free of extraneous bonding agents, the plate having a density such as corresponds in a plate of 60 pound ream weight and 0.004 inch thickness to an opacity of from 0.45 to 0.60, the sheet material which forms the printing surface being readily wet by and absorptive of water applied to the printing surface, so as to repel printing ink in the non-imaged areas under printing conditions, but the printing surface having a lateral water diffusion rate of not more than 25 millimeters in four hours.

2. A parchmentized cellulose planographic printing plate, the printing surface thereof having planographic printing characteristics, and the plate consisting of two superposed sheets of parchmentized cellulose, a continuum of non-fibrous amyloid cellulose extending throughout both sheets, said continuum overlaying the fibers near each face of the plate and also constituting a fiber-free and dense stratum at the junction between the two sheets, said junction stratum integrally uniting the two constituent sheets and being free of extraneous bonding agents, the sheet which forms the printing surface portion of the plate being of wood origin containing

traces of resinous material, and said resinous material being in an immobile state to prevent it from migrating to the printing face and thereby causing autogenous ink-receptive spotting.

3. A parchmentized cellulose planographic printing plate, the printing surface thereof having planographic printing characteristics, and the plate being formed of two superposed sheets of parchmentized cellulose, a continuum of non-fibrous amyloid cellulose extending throughout both sheets, said continuum overlaying the fibers near each face of the plate and also constituting a fiber-free and dense stratum at the junction between the two sheets, said junction stratum integrally uniting the two constituent sheets and being free of extraneous bonding agents, the plate having a density such as corresponds in a plate of 60 pound ream weight and 0.004 inch thickness to an opacity of from 0.45 to 0.60.

4. A parchmentized cellulose planographic printing plate, the printing surface thereof having planographic printing characteristics, and the plate being formed of two superposed sheets of parchmentized cellulose, a continuum of non-fibrous amyloid cellulose extending throughout both sheets, said continuum overlaying the fibers near each face of the plate and also constituting a fiber-free and dense stratum at the junction between the two sheets, said junction stratum integrally uniting the two constituent sheets and being free of extraneous bonding agents, the sheet material which forms the printing surface being readily wet by and absorptive of water applied to the printing surface, so as to repel printing ink in the non-imaged areas under printing conditions, but the lateral water diffusion rate of the printing surface being not more than 25 millimeters in four hours.

5. A parchmentized cellulose planographic printing plate, the printing surface thereof having planographic printing characteristics, and the plate consisting of two superposed fibrous sheets of parchmentized cellulose, a continuum of non-fibrous amyloid cellulose extending throughout the plate, said continuum overlaying the fibers near each face of the plate and also constituting a fiber-free and dense bonding stratum at the junction between the two sheets, said bonding stratum integrally uniting the two constituent sheets and being free of extraneous bonding agents, and an ink-receptive image on said printing surface and adapted to be retained by said surface when water is subsequently applied thereto in use of the plate.

6. A parchmentized cellulose planographic printing plate, the printing surface thereof having planographic printing characteristics, and the plate consisting of two superposed fibrous sheets of parchmentized cellulose, a continuum of non-fibrous amyloid cellulose extending throughout the plate, said continuum overlaying the fibers near each face of the plate and also constituting a fiber-free and dense bonding stratum at the junction between the two sheets; said

bonding stratum integrally uniting the two constituent sheets and being free of extraneous bonding agents, the plate having a thickness of approximately 0.004 inch, and an ink-receptive image on said printing surface and adapted to be retained by said surface when water is subsequently applied thereto in use of the plate.

7. A parchmentized cellulose planographic printing plate, the printing surface thereof having planographic printing characteristics, and the plate being formed of two superposed sheets of parchmentized cellulose, a continuum of non-fibrous amyloid cellulose extending throughout both sheets, said continuum overlaying the fibers near each face of the plate and also constituting a fiber-free and dense stratum at the junction between the two sheets, said junction stratum integrally uniting the two constituent sheets and being free of extraneous bonding agents, the plate having a density such as corresponds in a plate of 60 pound ream weight and 0.004 inch thickness to an opacity of from 0.45 to 0.60, and an ink-receptive image on said printing surface and adapted to be retained by said surface when water is subsequently applied thereto in use of the plate.

8. A parchmentized cellulose planographic printing plate, the printing surface thereof having planographic printing characteristics, and the plate consisting of two superposed fibrous sheets of parchmentized cellulose, a continuum of non-fibrous amyloid cellulose extending throughout the plate, said continuum overlaying the fibers near each face of the plate and also constituting a fiber-free and dense bonding stratum at the junction between the two sheets, said bonding stratum integrally uniting the two constituent sheets and being free of extraneous bonding agents, the density of the two constituent sheets of the plate being substantially the same, and an ink-receptive image on said printing surface and adapted to be retained by said surface when the water is subsequently applied thereto in use of the plate.

45 9. A parchmentized cellulose planographic printing plate, the printing surface thereof having planographic printing characteristics, and the plate consisting of two superposed fibrous sheets of parchmentized cellulose, a continuum of non-fibrous amyloid cellulose extending throughout the plate, said continuum overlaying the fibers near each face of the plate and also constituting a fiber-free and dense bonding stratum at the junction between the two sheets, said bonding stratum integrally uniting the two constituent sheets and being free of extraneous bonding agents, the plate having a ream weight of approximately 60 pounds, and an ink-receptive image on said printing surface and adapted to be retained by said surface when water is subsequently applied thereto in use of the plate.

WILLIAM B. WEScott.